

# UNITED STATES PATENT OFFICE.

CHARLES DEAR, OF LONDON, ENGLAND, ASSIGNOR TO THE MIRIS STEEL COMPANY  
LIMITED, OF LONDON, ENGLAND.

## MANUFACTURE OF STEEL.

1,304,946.

Specification of Letters Patent.

Patented May 27, 1919.

No Drawing.

Application filed December 30, 1916. Serial No. 139,908.

To all whom it may concern:

Be it known that I, CHARLES DEAR, a subject of the King of England, residing in London, England, have invented certain new and useful Improvements in the Manufacture of Steel, of which the following is a specification.

This invention relates to that procedure in the manufacture of steel by which the steel is immersed hot in a bath of liquid with a view to improving the constitution of the steel by means of the reactions taking place between it and the materials in the bath.

According to the present invention the liquid for a bath of the kind described contains nitric acid, sulfuric or alternatively sulfurous acid and an ammonium compound, such for example as ammonium hydrate or ammonium chlorid. If desired the two sulfur acids may both be used. The preferred composition of bath is one in which ammonium hydrate is employed, whether alone or in conjunction with ammonium chlorid or some other ammonium compound.

The bath is most effectual if the steel is immersed in it at a temperature of not less than about 800° C. at its outer surface.

The proportions in which the said materials are employed are preferably those of the following weights of each added to each thousand gallons of water, namely 2 cwt. of sulfuric or sulfurous acid; 3 cwt. of nitric acid;  $2\frac{1}{2}$  cwt. of sal-ammoniac. Or I may use 1 cwt. of sulfuric and 1 cwt. of sulfurous acid instead of 200 cwt. of sulfuric or sulfurous acid. It is preferred, further, to add  $2\frac{1}{2}$  cwt. of strongest liquid ammonia to each thousand gallons of water. After repeated use this last ingredient should be added to restore vigor of operation to the bath and in proportion as this is added so should also the nitric, sulfuric or sulfurous acid be added maintaining the aforestated proportions, that is to say, two and three parts, by weight respectively of the acids to  $2\frac{1}{2}$  parts by weight of the liquid ammonia.

The bath is prepared by dissolving first in the water such solids as are employed, then adding the liquids, the liquid ammonia being added last of all. As the fluid evaporates water should be added to make good this loss and as the bath loses ammonia this loss also should be made good, taking care to add also the other ingredients if and when

necessary to preserve the constitution of the bath in the proportions stated.

The valuable effects of immersing steel in this bath are realized to the best of advantage if the steel be plunged in it at a temperature at which the interior of the mass is still fluid or partly fluid, or if it be not convenient to operate before the temperature has sunk below this value, for want of facilities so to do, then the temperature should be again raised so as to be not less than that at which the interior will be fluid or nearly fluid. In any case the effects are less marked or penetrate to a less depth if the mass has been reduced in area by rolling or otherwise subjected to mechanical working.

The steel should not be removed from the bath except to be put into the soaking pits until recalescence cannot occur in the open air after removal.

Although the hereinbefore indicated conditions of use are those which enhance the valuable effects of this invention, the application of this invention is not limited to cases in which the said conditions obtain. The hereinbefore described bath for the immersion of hot steel to change and improve its qualities, other than to harden it by the ordinary process of plunging the steel to cool it suddenly, is a bath within the scope of the present invention, however used.

It has heretofore been proposed to treat steel with gas, fluids, or solids, in order to introduce hydrogen thereinto and such processes have been applied to high carbon and low carbon steel; it has furthermore been proposed to immerse billets or other rolled sections in various liquid compounds.

The general effect of this bath is to enhance the toughness of the steel and its ductility. The process is applicable, with advantageous results to alloy steels, such, for example, as nickel steel.

What I claim as my invention and desire to secure by Letters Patent is:—

1. An aqueous liquid for quenching hot steel to improve its toughness or its ductility which liquid contains nitric acid, a sulfur acid and an ammonium compound.

2. An aqueous liquid for quenching hot steel to improve its toughness or its ductility which liquid has been prepared by mixing nitric acid, sulfuric or sulfurous acid, an ammonium compound and water.

3. An aqueous liquid for quenching hot

steel to improve its toughness or its ductility which liquid contains nitric acid, a sulfur acid and an ammonium compound in the proportions of 3 cwt. of the nitric acid, 2 cwt. of sulfur acid and  $2\frac{1}{2}$  cwt. of ammonium chlorid to every 1000 gallons of water.

5 4. The method of treating steel comprising the step of placing a piece of hot steel in a bath containing nitric acid, sulfur acid and an ammonium compound.

10 5. The method of treating steel comprising the step of plunging a piece of steel in which the interior is still molten into a bath containing nitric acid, sulfur acid and an ammonium compound.

15 6. The method of treating steel comprising the step of plunging a piece of steel in which the interior is still molten into a bath containing nitric acid, sulfuric acid and an ammonium compound.

20 7. The method of treating steel comprising

ing the step of providing a bath containing 3 cwt. of nitric acid, 2 cwt. of sulfur acid, and  $2\frac{1}{2}$  cwt. of ammonium chlorid to every 1000 gallons of water, and plunging a piece 25 of hot steel in said bath and retaining it therein until it has become cold beyond the point where recalescence cannot occur in the open air after removal.

8. The method of treating steel comprising the step of providing a bath containing 3 cwt. of nitric acid, 2 cwt. of sulfur acid, and  $2\frac{1}{2}$  cwt. of ammonium chlorid to every 1000 gallons of water, and plunging a piece 30 of steel which has been heated to a tempera- 35 ture of 800° C. into said bath and retaining it therein until it has become cold beyond the point where recalescence cannot occur in the open air after removal.

In testimony whereof I have signed my 40 name to this specification.

CHARLES DEAR.

Copies of this patent may be obtained for five cents each, by addressing the "Commissioner of Patents, Washington, D. C."